

Patented Mar. 24, 1925.

## UNITED STATES PATENT OFFICE.

ROBERT M. ISHAM, OF OKMULGEE, OKLAHOMA, ASSIGNOR, BY MESNE ASSIGNMENTS,  
TO SETH B. HUNT, TRUSTEE, OF MOUNT KISCO, NEW YORK.

## FLOTATION OIL.

No Drawing.

Application filed December 17, 1921. Serial No. 523,205.

To all whom it may concern:

Be it known that I, ROBERT M. ISHAM, a citizen of the United States of America, residing at Okmulgee, in the county of 5 Okmulgee, State of Oklahoma, have invented certain new and useful Improvements in Flotation Oils; and I do hereby declare the following to be a full, clear, and exact description of the invention, such as 10 will enable others skilled in the art to which it appertains to make and use the same.

This invention relates to flotation oils and more particularly to a method of concentrating ores by froth flotation and re- 15 agents for producing the flotation froth.

The well-known flotation process of concentrating ores consists in separating metalliferous matter, particularly metallic sulphides, from the gangue of the ore. By 20 this process pulverized ore is thoroughly mixed with water containing a small amount of a frothing agent, and the mixing is so conducted as to thoroughly aerate the mixture to coat the metalliferous matter with air bubbles and to form a froth. The froth carries the metal and may be readily separated from the water carrying the gangue to recover the metal. A large 25 number of different kinds of frothing agents have been used for floating metalliferous matter, and it has been found that different kinds of metals and ores require different kinds and quantities of frothing agents. A careful study of the physical 30 phenomena involved in the flotation of metallic matter shows that two distinct properties are required of a flotation oil to obtain the desired results:—First, a portion of the oil must be dissolved in water and act to diminish the surface tension of the water, and second, a part of the oil must remain undissolved and act to coat the surface of the metallic particles to float and collect them.

The primary object of the present invention is to provide a flotation oil which has desirable properties for making a full and efficient separation of the metalliferous matter from the gangue of the ore.

Another object of the invention is to provide a flotation oil which may be modified readily to be adapted for treating any of the various kinds of ore, and for treating other products by flotation processes.

With these and other objects in view, the

invention consists in the improved flotation oils hereinafter described and particularly defined in the claims.

In the copending application of Sidney Born and Robert M. Isham, Serial No. 294,013, filed May 1, 1919, for "process of producing alcohols," is described a process by which alcohols, polymerized olefines, alkyl hydrogen sulphates and other products can be manufactured from oil gas. In accordance with this process, oil gas which preferably is obtained by cracking oil under pressure, is scrubbed under pressure by a countercurrent circulation with a solution containing concentrated sulphuric acid and alkyl hydrogen sulphates. By this scrubbing operation the olefines are selectively sulphated at different temperatures. The higher olefines such as hexylene, amylene and butylene, are absorbed at temperatures below 0° C. The propylene is absorbed at a temperature of about 20° C. and the ethylene is absorbed at a temperature of about 80 to 90° C. The acid liquor delivered from the absorbers contains alkyl hydrogen sulphates, sulphuric acid, polymerized olefines and diolefines, saturated and unsaturated hydrocarbons. The condensed unabsorbed hydrocarbons are not miscible in the acid liquid and may be separated therefrom by gravity separation. By diluting the acid liquid with water the alkyl hydrogen sulphates are partially hydrated and the polymerized unsaturated hydrocarbons are set free and may be separated therefrom by a gravity separation. The hydrolyzation of the acid liquid may be completed in a fractionating still and by properly fractionating and rectifying the said liquid, the various alcohols may be collected separately. Also groups or mixtures of alcohols may be collected by appropriate fractional distillation.

The polymerized unsaturated hydrocarbons obtained by the process outlined above are collected in the form of an oil which has a dark green or brown color which is opalescent. This oil is not a tar and does not ordinarily contain tar. In this respect it may be clearly distinguished from the sludge that is recovered in the ordinary methods of treating petroleum distillates with concentrated sulphuric acid at ordinary temperatures to decolorize and deodorize them. The oil contains polymerized simple and higher olefines, polymerized diolefines or

unsaturated hydrocarbons with two double linkings, polymerized acetylene or hydrocarbons with triple linkings, and some other unsaturated hydrocarbons. The percentage 5 composition of the various types of unsaturated hydrocarbons in the polymerized oil depends upon the character of the oil gas from which the oil is made. If the oil is cracked under pressure at extremely high 10 temperatures, a comparatively high percentage of diolefines will be formed. If a large percentage of the diolefines is present, the oil may contain some tars because the diolefines react so readily with concentrated 15 sulphuric acid that it is difficult to prevent the formation of tars. When oil is cracked at the comparatively lower temperatures and pressure, that is, 100 pounds pressure or lower, and 800° F. or lower, a small 20 amount of diolefines is formed in the oil gases, and these may be readily polymerized without the formation of tars. The polymerized oils formed from gases produced 25 when cracking oil at the lower pressures and temperatures, contain a major portion of the polymerized simple olefines.

All of the oils described above which contain polymerized unsaturated hydrocarbons (hereinafter termed "polymerized oils") 30 have remarkable collecting properties for selecting the metalliferous matter of the ore and coating it with an oily film in preference to coating the gangue. In addition to having the collective property, it is necessary 35 for a successful flotation oil to have froth forming properties. With some forms of ores the polymerized oils will form very satisfactory froths, and can be used alone. With this purpose, the polymerized oil has 40 been used in the proportion of 1% to 1/20 of 1% of the weight of the ore being treated, and gives very satisfactory flotation results.

In order to obtain a maximum selective 45 action between sulphide minerals and a gangue of the mineral, it is necessary to have the greatest possible difference between the properties of the water phase and the oil phase in the flotation system. The polymerized oil may be considered as practically 50 insoluble in water; hence it will produce the greatest possible difference between water phase and the oil phase, and consequently give a greater selective action. In case where the polymerized oils do not produce 55 a satisfactory froth, it has been found that the addition of an alcohol will give this result, particularly the alkyl alcohols which are produced by the Born and Isham process outlined above.

60 An examination of the various alcohols produced from oil gases shows that there is a steadily decreasing solubility with the increase in molecular weight and with the passage from the tertiary to the secondary 65 and then to the primary alcohols. The

lighter alcohols, such as ethyl and propyl alcohol can be considered as practically fully soluble in water, while the heavier alcohols become less and less soluble as their molecular weights increase.

When a flotation oil, which is made up by polymerized oil and a heavy alcohol that is only slightly soluble in water, is used in a water menstruum, the alcohol will be distributed between the water phase and the 70 polymerized oil phase. The greater the amount of alcohol associated with the water phase, the closer will be the similarity in the property of the oil and water phases, and the selective action of 75 the polymerized oil will be relatively diminished. It will be seen therefore that by the use of the polymerized oil and alcohols which have different degrees of solubility in water, a flotation oil of practically any desired combination of selective and froth forming properties may be obtained.

By means of the Born and Isham process of producing alcohols from oil gas, the following more simple aliphatic alcohols may be produced; ethyl alcohol, secondary propyl, butyl, amyl, hexyl and heptyl alcohols, and tertiary, butyl, amyl, hexyl and heptyl alcohols. Tests which have been 90 made with these various alcohols have shown that all of them except ethyl will produce a satisfactory froth for a flotation process. Further, there is a continuous increase in the depths of froth which will be formed 95 by the alcohols as the molecular weights of the alcohol increase. It is not necessary that these aliphatic higher alcohols shall be produced by the Born and Isham process described above, and tests have been made with 100 the commercial aliphatic higher alcohols which show that they produce very satisfactory froths. In working out various combinations of alcohols with polymerized oils, it is found that the greater the molecular 105 weight of the alcohols, the smaller is the proportion of the polymerized oil required 110 in order to produce the maximum depth of froth.

Tests have shown that the higher aliphatic 115 alcohols not only possess frothing properties for flotation oil, but also possess selective properties, and therefore the higher alcohols may be used alone and give a satisfactory metal separation. For example, tertiary 120 butyl and tertiary amyl alcohols will give a satisfactory separation of the metal sulphides of the zinc sulphide ores. It is also possible to combine with some of the higher 125 insoluble aliphatic alcohols, one or more of the lower aliphatic alcohols which are slightly soluble in water to thus modify the selective and frothing properties of the oil.

Below are given examples of flotation 130 oils which have been satisfactory used in

connection with separating the metalliferous matter of the sphalerites, chalcopyrites, copper sulphides, zinc blends and the galena ores:

- 5 1. Polymerized oil 2 parts. Iso propyl alcohol 1 part.  
2. Polymerized oil 2 parts. Tertiary butyl alcohol 1 part.  
3. Polymerized oil 4/5 parts. Secondary butyl alcohol 1 part.

- 10 4. Polymerized oil 3/10 parts. Mixed secondary and tertiary amyl alcohols 1 part.

- 15 5. Polymerized oil 2/5 parts. Commercial iso butyl alcohol 1 part.  
6. Polymerized oil 3/5 parts. Commercial secondary and tertiary alcohol 1 part.

These flotation oils have been used in the ratio of 1/20 of one per cent to one per cent by weight of the ore being treated, the proportion of the flotation oil depending upon the character of the ore. It has also been found that the presence of an acid with the flotation oil will sometimes assist in preventing the gangue from being coated with

25 the oil and thus allow the flotation oil to be more effective in floating the metalliferous metal. Therefore, a small amount of free sulphuric acid or alkyl sulphuric acid has been used with a flotation oil consisting of 30 polymerized oil alone, or consisting of polymerized oil with an alcohol or a mixture of alcohols, or consisting of an alcohol alone or a mixture of alcohols.

Although the invention has been described 35 by reference to the use of polymerized unsaturated hydrocarbon oils, and the various aliphatic alcohols which are particularly produced by the process of Born and Isham, the invention is not limited to the use of 40 the polymerized oils and alcohols produced by this process, but any of the various polymerized oils and aliphatic alcohols which are produced by any of the known processes may be used in making a flotation product.

45 The preferred form of the invention having been thus described, what is claimed as new is:

1. As an article of manufacture an oil-like product comprising a mixture of polymerized hydrocarbons and alcohol.

2. As an article of manufacture an oil-like product comprising a mixture of polymerized unsaturated hydrocarbons and alcohol.

3. As an article of manufacture an oil-like product comprising a mixture of polymerized hydrocarbons and higher aliphatic alcohol. 55

4. As an article of manufacture an oil-like product comprising a mixture of polymerized unsaturated hydrocarbons and a secondary alcohol. 60

5. As an article of manufacture an oil-like product comprising a mixture of polymerized unsaturated hydrocarbons and a mixture of secondary alcohols. 65

6. As an article of manufacture an oil-like product comprising a mixture of polymerized unsaturated hydrocarbons and a tertiary alcohol. 70

7. As an article of manufacture an oil-like product comprising a mixture of polymerized unsaturated hydrocarbons and a mixture of tertiary alcohols.

8. As an article of manufacture an oil-like product comprising a mixture of polymerized olefines and diolefines. 75

9. As an article of manufacture an oil-like product comprising a mixture of polymerized olefines and diolefines and higher aliphatic alcohol. 80

10. As an article of manufacture an oil-like product comprising a mixture of polymerized unsaturated hydrocarbons and alkyl hydrogen sulphate. 85

11. As an article of manufacture an oil-like product comprising a mixture of polymerized olefines and higher aliphatic alcohol.

12. As an article of manufacture an oil-like product comprising a mixture of polymerized olefines and diolefines, secondary and tertiary alcohols, and alkyl hydrogen sulphate. 90

13. As an article of manufacture a flotation oil comprising not less than ten per cent by volume of polymerized unsaturated hydrocarbon constituents.

In testimony whereof I affix my signature.

ROBERT M. ISHAM.